

1

2,867,518

## DETONATOR COMPOSITIONS

David T. Zebree, Kingston, N. Y., assignor to Hercules Powder Company, Wilmington, Del., a corporation of Delaware

No Drawing. Application December 31, 1956  
Serial No. 631,469

20 Claims. (Cl. 52—2)

This invention relates to initiator compositions. In one aspect this invention relates to lead-tellurium compositions, containing fatty acid salts, as blasting initiators. In another aspect this invention relates to lead-tellurium compositions, containing fatty acid salts, particularly suitable as ignition mixtures in electric blasting caps. In still another aspect this invention relates to lead-tellurium-fatty acid salt compositions as ignition materials and containing selected additives for the regulation of their fuse ignitability characteristics when employed as igniters in delay caps.

Blasting cap charges comprise generally a base charge of a detonating explosive such as pentaerythritol tetrinitrate, a heat-sensitive primer charge such as diazodinitrophenol, mercury fulminate or lead azide superposed on the base charge, and a readily ignitable ignition charge capable of firing the primer charge by the heat generated. In the case of delay caps an additional slow burning composition or delay fuse is generally included between the ignition and primer charges and exhibits such a predetermined rate of burning that the specified time interval elapses between the application of the firing current and the explosion of the primer charge.

This invention is concerned with new blasting initiator compositions advantageously applied as ignition charges in electric blasting caps. The said charges are also applicable as delay fuses in certain applications.

An object of this invention is to provide new blasting initiators. Another object is to provide new compositions especially suitable as ignition charges in blasting caps. Still another object is to provide ignitable lead-tellurium-fatty acid salt compositions containing an additive comprising one or more selected materials to regulate their fuse ignitability characteristics when employed as initiators in a delay cap. Other aspects and objects will be apparent from the accompanying disclosure and the appended claims.

In accordance with this invention lead-tellurium compositions containing lead and tellurium in ignitable pro-

portions, together with a minor amount of a metal salt of a long chain fatty acid, are provided as blasting initiators. Further in accordance with this invention lead-tellurium compositions are provided which contain lead and tellurium in ignitable proportions, together with a minor proportion of a metal salt of a long chain fatty acid, and at least one additive capable of altering the fuse ignitability characteristics of the said composition when utilized as an initiator in a blasting cap and selected from the group of magnesium, aluminum, silicon, phosphorus and sulfur. Still in accordance with this invention a method is provided for regulating firing time of a blasting cap which comprises firing a blasting cap containing a lead-tellurium ignition mixture and regulating the time of said firing by maintaining a sufficient amount of a metal salt of a long chain fatty acid in the said mixture to decrease the said firing time to a predetermined value.

Although it is within the scope of my invention to utilize any ignitable proportions of lead and tellurium in my compositions, the preferred composition will contain from about 35 to 81 weight percent lead and from about 19 to 65 weight percent tellurium. The amount of long chain fatty acid salt, as discussed more fully hereinafter, will generally be within the range of about 0.1 to 6 weight percent. The amount of additive component utilized depends upon the problem at hand, being, however, in the order of from about 0.3 up to 4.5 weight percent or higher if desired. Substantially stoichiometric proportions of lead and tellurium are employed in my compositions to achieve maximum heat of reaction, which is of particular importance in the use of the composition as an ignition mixture in a delay cap in order to assure ignition of the fuse. However, other than stoichiometric proportions can be employed for that purpose when desired, particularly when an additive material is present to increase the fuse ignitability by increasing the heat of the burning reaction as described hereinafter.

The following tabulation of data are illustrative of firing time obtained with lead-tellurium-fatty acid salt compositions of this invention as detonator compositions in short-period delay caps, there being no separate delay charge present. Also included are firing time data obtained with lead-tellurium-fatty acid salts containing silicon. Firing time data, illustrative of lead-tellurium mixtures alone, are included for comparison. The data illustrate the regulatory effect of the fatty acid salt components of this invention on the burning rate of lead-tellurium mixtures. The base charge and primer compositions employed were pentaerythritol tetrinitrate and diazodinitrophenol, respectively, in conventional proportions. The lead-tellurium proportions were 61.9/38.1 in all cases. All tests were made in a standard 25 caliber shell.

Table I

| Ignition mixture                  | Weight of ignition or delay charge, grams | Number of tests | Summary of firing time (milliseconds) |         |        |
|-----------------------------------|-------------------------------------------|-----------------|---------------------------------------|---------|--------|
|                                   |                                           |                 | Avg.                                  | Range   | Spread |
| Pb—Te                             | 0.7                                       | 10              | 163                                   | 55-185  | 130    |
| Pb—Te/Pb stea. 1/Sl. 97.5/1.5/1.0 | 0.7                                       | 10              | 44                                    | 35-55   | 20     |
| Pb—Te/Pb stea. 1/99.1             | 0.7                                       | 10              | 45                                    | 40-50   | 10     |
| Pb—Te/Pb stea. 1/98.5/1.5         | 0.7                                       | 10              | 45                                    | 40-55   | 15     |
| Pb—Te/Pb stea. 1/98.2             | 0.7                                       | 10              | 50                                    | 40-75   | 35     |
| Pb—Te                             | 1.4                                       | 10              | 440                                   | 200-620 | 420    |
| Pb—Te/Pb stea. 1/Sl. 97.5/1.5/1.0 | 1.4                                       | 10              | 70                                    | 60-85   | 20     |
| Pb—Te/Pb stea. 1/99.1             | 1.4                                       | 8               | 67                                    | 60-75   | 15     |

\* Lead stearate.

The following tabulation of data are illustrative of firing times obtained with lead-tellurium-fatty acid metal salt-silicon compositions of this invention with additive components as ignition mixtures in a delay cap containing a delay fuse. Firing time data illustrative of lead-tellurium mixtures are included for comparison.

admixed by any suitable procedure. Generally the particle size of the resulting composition will be in the range of about 1 to 70 microns, although a particle size outside that range can be utilized if desired. The composition is loaded into any desired form of blasting cap in any usual manner. No air space is required in the cap since

Table II

| Ignition mix. (loose)                | Fuse powder                                                         | Number of tests | Fuse length, inches | Firing time (ms.) |           |        |
|--------------------------------------|---------------------------------------------------------------------|-----------------|---------------------|-------------------|-----------|--------|
|                                      |                                                                     |                 |                     | Avg.              | Range     | Spread |
| Pb-Te <sup>1</sup>                   | BaO <sub>2</sub> Te(70-30)/PbSn, 50/50                              | 10              | 0.192               | 470               | 420-1,000 | 580    |
| Pb-Te <sup>1</sup>                   | BaO <sub>2</sub> Te(70-30)/PbSn, 50/50                              | 10              | 0.334               | 770               | 700-1,950 | 1,250  |
| Pb-Te 1/Pb stearate/Si, 97.5/1.5/1.0 | BaO <sub>2</sub> Te(70-30)/PbSn, 50/50                              | 10              | 0.093               | 210               | 195-250   | 55     |
| Pb-Te 1/Pb stearate/Si, 97.5/1.5/1.0 | BaO <sub>2</sub> Te(70-30)/PbSn, 50/50                              | 10              | 0.192               | 395               | 360-420   | 60     |
| Pb-Te 1/Pb stearate/Si, 97.5/1.5/1.0 | BaO <sub>2</sub> Te(70-30)/PbSn, 50/50                              | 10              | 0.334               | 670               | 640-690   | 50     |
| Pb-Te <sup>1</sup>                   | Pb-Se <sup>2</sup> /BaO <sub>2</sub> -Se(82-18); 70/30 <sup>3</sup> | 10              | -----               | 368               | 280-500   | 220    |
| Pb-Te 1/Pb stearate/Si, 97.5/1.5/1.0 | Pb-Se <sup>2</sup> /BaO <sub>2</sub> -Se(82-18); 70/30 <sup>3</sup> | 10              | -----               | 90                | 75-100    | 25     |
| Pb-Te 1/Pb stearate/Si, 97.5/1.5/1.0 | BaO <sub>2</sub> /Se(75-25) <sup>4</sup>                            | 10              | -----               | 395               | -----     | 60     |
| Pb-Te 1/Pb stearate/Mg, 97.5/1.5/1.0 | BaO <sub>2</sub> /Se(75-25) <sup>4</sup>                            | 10              | -----               | 400               | -----     | 20     |

<sup>1</sup> Stoichiometric proportions (61.9-38.1).

<sup>2</sup> Stoichiometric proportions (72.4-27.6).

<sup>3</sup> Pressed (0.7 gram) on primer charge.

<sup>4</sup> Pressed (0.65 gram) on primer charge.

The foregoing examples demonstrate that metal fatty acid salt components of the compositions of this invention provide for improved firing accuracy as manifest by the lowered spread in firing times of lead-tellurium mixtures that is achieved, and for marked reduction in firing time of lead-tellurium ignition mixtures to provide for regulation of those firing times to significantly reduced values. The additive components, namely magnesium, silicon, aluminum, sulfur and phosphorus impart increased heat of reaction to provide supplemental heat for igniting difficultly ignitable delay fuses in blasting caps.

While any metal salt of the long chain fatty acids can be employed in the practice of my invention, the stearates, oleates, laurates, caprates, caprylates, and palmitates are advantageously employed. Further illustrative of the fatty acid salt components of this invention are: lead stearate, cadmium stearate, iron stearate, magnesium stearate, aluminum stearate, zinc stearate, calcium stearate, lead laurate, cadmium laurate, iron laurate, magnesium laurate, aluminum laurate, zinc laurate, calcium laurate, lead palmitate, cadmium palmitate, iron palmitate, magnesium palmitate, aluminum palmitate, zinc palmitate, calcium palmitate, lead caprylate, lead caprate, cadmium caprylate, cadmium caprate, iron caprylate, iron caprate, magnesium caprylate, aluminum caprylate, zinc caprylate, calcium caprylate, magnesium caprate, aluminum caprate, zinc caprate and calcium caprate. Lead stearate is the preferred fatty acid salt component of the compositions of this invention.

The amount of fatty acid salt in my compositions is sufficient to impart improved accuracy of burning lead-tellurium mixtures. Lead-tellurium mixtures as blasting initiators, together with additive materials therefor when desired and certain method aspects relating thereto, are disclosed and claimed in my copending application Serial No. 631,467, filed December 31, 1956.

The above-described amount of fatty acid salt component is generally within the range of about 0.1 to 6 weight percent of the composition although 0.2 to 2 percent is preferred. The upper limit in any event is not above that which will undesirably desensitize the composition to ignition, the above maximum value depending largely upon the specific metal salt and the firing current utilized.

The compositions of this invention will burn without the production of any substantial amount of gas and thus will not rupture the cap casing or dislodge the bridgewire upon firing. In preparing a composition of this invention in accordance with one embodiment, the ingredients are reduced to a finely-divided form and are then intimately

the composition develops practically no gas on burning.

As illustrative, the composition may be loaded loosely into any form of ventless delay cap assembly above the fuse and the usual sulfur plug holding the usual bridgewire placed above the loosely loaded composition with the bridgewire embedded in the composition. Similarly, a composition may be loosely loaded into any ordinary blasting cap above the priming charge.

As will be evident to those skilled in the art, various modifications can be made or followed, in the light of the foregoing disclosure and discussion, without departing from the spirit or scope of the disclosure or from the scope of the claims.

What I claim and desire to protect by Letters Patent is:

1. As a blasting initiator composition, an ignition mixture of lead and tellurium containing a metal salt of a long chain fatty acid in an amount sufficient to decrease the burning time of said lead and tellurium but less than that which completely desensitizes the said composition to ignition, whereby spread in burning time of said lead and tellurium is also decreased.

2. A composition of claim 1 containing a sufficient amount of at least one additive selected from the group consisting of aluminum, magnesium, silicon, sulfur and phosphorus to impart increased heat of reaction from burning of said composition.

3. As a new composition a finely divided blasting initiator mixture consisting essentially of from 35 to 81 weight percent lead, from 19 to 6.5 weight percent tellurium and from 0.1 to 6 weight percent of a metal salt of a long chain fatty acid.

4. A composition of claim 3 wherein said lead and tellurium are present in substantially a lead/tellurium weight ratio of 61.9:38.1.

5. A new composition consisting essentially of a finely divided blasting initiator mixture of from 35 to 81 weight percent lead, from 19 to 65 weight percent tellurium, from 0.1 to 6 weight percent of a metal salt of a long chain fatty acid, and from 0.3 to 4.5 weight percent of at least one additive of the group of aluminum, magnesium, silicon, sulfur and phosphorus.

6. A composition of claim 5 wherein said additive is silicon.

7. A composition of claim 5 wherein said additive is magnesium.

8. A composition of claim 5 wherein said additive is aluminum.

9. A composition of claim 5 wherein said additive is sulfur.

10. A composition of claim 5 wherein said additive is phosphorus.

11. In an electric blasting cap containing a detonatable base charge and a primer charge for initiating said base charge upon being heated, and an ignition charge for generation of heat, from burning of same, to cause initiation of said primer, the improvement providing, as said ignition charge, an ignition mixture of lead and tellurium containing a metal salt of a long chain fatty acid in an amount sufficient to decrease the burning time of said lead and tellurium but less than that which completely desensitizes the said composition to ignition.

12. A cap of claim 11 wherein said charge contains at least one of magnesium, aluminum, silicon, sulfur and phosphorus as an additive in an amount sufficient to impart increased heat of reaction from burning of said ignition charge.

13. A composition of claim 1 wherein said metal salt is a stearate.

14. A composition of claim 3 wherein said fatty acid is of the group of stearic, oleic, lauric, capric, caprylic and palmitic.

15. As a new blasting initiator composition a finely divided mixture consisting essentially of from 35 to 81 weight percent lead, 19 to 65 weight percent tellurium, and from 0.2 to 2 weight percent of a metal salt of a long chain fatty acid.

16. A composition of claim 15 wherein said salt is lead stearate.

17. A blasting cap of claim 11 wherein the said ignition charge is the sole ignitable charge for initiating said primer.

18. A blasting cap of claim 17 wherein said charge contains at least one of magnesium, aluminum, silicon, sulfur and phosphorus as an additive in an amount sufficient to impart increased heat of reaction from burning of said ignition charge.

19. As a new blasting initiator composition, a finely divided mixture consisting essentially of from 35 to 81 weight percent lead, from 19 to 65 weight percent tellurium, from 0.2 to 2 weight percent lead stearate, and from 0.3 to 4.5 percent silicon.

20. As a new blasting initiator composition, a finely divided mixture consisting essentially of from 35 to 81 weight percent lead, from 19 to 65 weight percent tellurium, from 0.2 to 2 weight percent lead stearate, and from 0.3 to 4.5 percent magnesium.

References Cited in the file of this patent

UNITED STATES PATENTS

|    |            |               |               |
|----|------------|---------------|---------------|
| 25 | Re. 19,661 | Nash          | July 30, 1935 |
|    | 2,146,033  | Seavey et al. | Feb. 7, 1939  |
|    | 2,370,159  | Hanley        | Feb. 27, 1945 |